

# UNITED STATES PATENT OFFICE.

WILLIAM J. LEDDELL, OF SUMMIT, NEW JERSEY.

## ALLOY.

No. 901,014.

Specification of Letters Patent.

Patented Oct. 13, 1908.

Application filed January 28, 1908. Serial No. 413,152.

To all whom it may concern:

Be it known that I, WILLIAM J. LEDDELL, a citizen of the United States, and residing at Summit, New Jersey, have invented a certain new and useful Improvement in Alloys, of which the following is a specification.

My invention relates to alloys, commonly known as zinc-alloys, and consisting principally of zinc, copper and aluminum, said alloys being particularly adapted for the production of light castings in iron molds, without the employment of expandible cores, and being especially suitable for various electrical and mechanical work, since a smooth finished casting may be obtained without machining. Owing to the fact that the rapidity of work is an important item in such construction, it is evident such an alloy is of no little importance for these purposes. Heretofore various alloys have been proposed in which the said ingredients were employed, but the slightest variation in proportions invariably resulted in the production of alloys possessing radically different properties, and in many instances the alloys produced were entirely unsuited for the purposes for which they were intended. For example, in alloys consisting principally of zinc, the introduction of copper in greater proportions than aluminum, produces an alloy whose melting point is relatively high and which, on cooling, shrinks to such an extent that the alloy, while possessing valuable anti-frictional properties, is entirely unsuited for a large variety of electrical and mechanical purposes, owing to its hardness and the difficulty of producing sharp and clearly defined castings in ordinary molds. On the other hand, when similar so-called zinc-alloys are employed, which contain aluminum in proportions in excess of the copper, a crystalline structure results, which is so susceptible in many instances to fracture, that when subjected to distortion strains by pressure or impact, it is liable to suddenly disintegrate without warning, thereby rendering the same not only impracticable for many purposes, but extremely dangerous.

This invention has for its objects the production of a so-called zinc-alloy, which, while melting at an extremely low temperature, possesses an extraordinary resistance to distortion by pressure or impact, and in such respects closely resembling iron, having a high conductivity and a high degree of fluid-

ity, and withal extremely light and possessing a remarkably low factor of shrinkage. In the production of said alloy a large proportion of zinc is employed, preferably 90 per cent. of the total weight of the alloy, being commercial zinc, which zinc often contains up to  $\frac{1}{16}$  per cent. of impurities in the form of iron and lead. Said zinc is alloyed in any desirable manner with equal proportions of aluminum and copper, preferably 5 per cent. of aluminum and 5 per cent. of copper. For special purposes, moreover, in order to increase the peculiar property of fluidity of the alloy, a very small percentage of cadmium may be employed, preferably less than  $\frac{1}{2}$  per cent., although ordinarily the employment of cadmium is unnecessary. The proportions of zinc may be varied in accordance with the requirements of the work for which the alloy is to be employed, but regardless of the amount of zinc introduced, the said zinc obviously being in all instances the principal ingredient of the alloy, equal amounts of aluminum and copper must be maintained in order to properly balance their respective properties and to produce an alloy corresponding to that herein described.

These alloys, especially that produced according to the preferred process herein detailed, are especially suitable for the production of light castings in iron molds, since no expandible core is required, even when standard threads are to be formed on said castings, and no machining of the same is subsequently necessitated.

Various nipples suitable for plumbing fixtures, journals, journal boxes, and in fact, as stated, various light castings, when produced from this alloy, are not only extremely economical, in so far as their production is concerned, but possess an attractive appearance somewhat resembling pure aluminum, and are extremely light in weight, while possessing a high degree of conductivity. The structure of the alloy is extremely dense and homogeneous, and substantially free from masses of crystallized zinc segregated throughout the mass. In use, there is a remarkable absence of corrosion of the metal, even when subjected to severe weathering, and moreover, there is an entire absence of any poisonous ingredients which would tend to render the same unsuitable for liquid-dispensing purposes.

In the claims the expression "consisting

principally of zinc" is used to define an alloy containing in excess of 85 per cent. of zinc, as it is apparent, that an alloy containing, for example, 60 per cent. of zinc and equal parts of copper and aluminum, would possess totally different properties from the alloys herein described and would be inapplicable for the special purposes for which these alloys are employed.

- 10 Owing to the various impurities occurring in the commercial articles which are employed in this alloy, and especially in the zinc and copper, the expression "substantially equal parts," as used in the claims, is 15 used to define proportions within variations of  $\frac{1}{4}$  of 1 per cent., as it is obviously impracticable in the commercial production of alloys to specify their proportions invariably within appreciably closer limits.
- 20 The expression "factor of shrinkage" as employed in the claims relates to the relative shrinkage of this alloy as compared with iron, and the alloy herein described in my preferred process of production possesses a 25 factor approximately .695 as compared with 1 for iron. It is evident that these figures are merely approximate, and that I do not limit the claims to the exact figure stated, as similar factors of shrinkage approximating 30 that of iron, although varying from the exact figures, *i. e.*, .695, are equally within the scope of my invention, since the closer approximation of the factor of shrinkage of

the alloy to that of iron, the more desirable will be the casting property. 35

Having thus described my invention, what I claim and desire to protect by United States Letters Patent is:

1. An alloy consisting principally of zinc, and containing substantially equal parts of aluminum and copper respectively, said alloy possessing a relatively low factor of shrinkage and a relatively high resistance to distortion from impact or pressure, and having a dense, homogeneous structure substantially 40 free from segregated masses of crystallized zinc.
2. An alloy containing in excess of eighty-seven and one-half per cent. of zinc, and containing substantially equal parts of aluminum and copper respectively. 50
3. An alloy consisting principally of zinc and containing substantially five per cent. of aluminum and five per cent. of copper.
4. An alloy containing substantially ninety 55 per cent. of zinc, five per cent. of aluminum and five per cent. of copper.

In testimony whereof, I have signed my name to this specification in the presence of two subscribing witnesses, this twenty-first 60 day of January, 1908.

WILLIAM J. LEDDELL.

Witnesses:

W. H. SWENARTON,  
ARTHUR M. SILBER.